

# UNITED STATES PATENT OFFICE.

GEORGE HENKEL AND HENRY HENKEL, OF LOGAN, OHIO.

## LIQUID SOAP.

SPECIFICATION forming part of Letters Patent No. 269,413, dated December 19, 1882.

Application filed October 28, 1882. (No specimens.)

*To all whom it may concern:*

Be it known that we, GEORGE HENKEL and HENRY HENKEL, citizens of the United States, residing at Logan, in the county of Hocking 5 and State of Ohio, have invented certain new and very useful Improvements in Liquid Soap, of which the following is a specification.

Our liquid soap consists of the following ingredients, combined in the proportions stated, 10 viz: Pure water, one hundred gallons; caustic soda, two hundred and seventy pounds; borax, thirty-five pounds; alum, four pounds, spirits of ammonia, two gallons. These ingredients, except the spirits of ammonia, are to 15 be placed over a fire in a proper vessel and heated until thoroughly mixed and combined. When this mixture is cold the spirits of am-

monia is to be added. Then the liquid soap should be drawn off into air-tight vessels to prevent evaporation, when it is ready for use 20 in quantities, according to direction.

Having thus fully described our said improvement, what we claim as our invention, and desire to secure by Letters Patent, is—

A liquid soap composed of one hundred gallons of pure water, two hundred and seventy pounds of caustic soda, thirty-five pounds of borax, four pounds of alum, and two gallons of spirits of ammonia. 25

GEORGE HENKEL.  
HENRY HENKEL.

Witnesses:

L. S. BORT,  
A. McCARTNEY.